

Dec. 14, 1926.

1,610,576

J. V. MOORE

DOUBLE WOVEN COLLAR FABRIC

Filed Jan. 23, 1924



Fig. 2



Fig. 3



Dividing Portion



Fig. 4



INVENTOR

John V. Moore

By Attorneys

Huntington & Huntington

Patented Dec. 14, 1926.

1,610,576

# UNITED STATES PATENT OFFICE.

JOHN V. MOORE, OF PAWTUCKET, RHODE ISLAND, ASSIGNOR, BY MESNE ASSIGNMENTS, TO VAN HEUSEN PRODUCTS, INC., A CORPORATION OF DELAWARE.

## DOUBLE-WOVEN-COLLAR FABRIC.

Application filed January 23, 1924. Serial No. 688,095.

This invention relates to a double woven fabric particularly adapted to the manufacture of soft or semi-soft collars for men's wear. As such collars are not strictly confined to a fixed form, it is desirable that they be given a natural and well defined fold line, so that they may assume the desired shape when in use.

It is the object of my invention to provide a multiple ply interwoven collar fabric in which the fold occurs adjacent the union or point of engagement of two different fabric portions having distinct characteristics. In the preferred form these fabric portions differ from each other in the size and spacing of the warp threads but not ordinarily in the structure of the weave.

A further object of my invention is to provide a multiple ply interwoven collar fabric in which a narrow intermediate folding portion is provided between the face portion and the band portion, this narrow intermediate portion differing from both other portions, either in the size or in the spacing of the warp threads.

A preferred form of the invention and two modifications thereof are shown in the drawings, in which—

Fig. 1 is a fragmentary plan view of a portion of my improved fabric;

Fig. 2 is a partial transverse sectional elevation taken along the line 2—2 in Fig. 1;

Fig. 3 is a partial longitudinal sectional elevation taken along the line 3—3 in Fig. 1;

Fig. 4 is a partial transverse sectional elevation of a modification, and

Fig. 5 is a similar view of a second modification.

Referring particularly to Figs. 1 and 3, I have shown a collar fabric which is preferably woven in curvilinear form and which comprises an outer or face portion 10 and an inner or band portion 11. As shown in Fig. 3, the fabric is of the multiple ply interwoven type, having face warps W, back warps W', a stuffer warp S, which may be omitted if desired, binder warps B and filling F. The stuffer warps S are shown in Figs. 2, 4 and 5 by the dotted circles lying between the two surface plies. The weave may be of the common form shown in Fig. 3 or may be varied to suit the requirements of a particular fabric.

A novel feature of my invention consists

in providing certain parts of the fabric with warp threads differing in size or spacing from the warp threads in other parts of the fabric. As illustrative of my invention, I have indicated in Fig. 1 an outer face portion formed with No. 80 threads, doubled and spaced 100 ends to the inch, while the back of this portion is formed of No. 30 threads, doubled and spaced 50 threads to the inch. Both inner and outer parts of the band portion 11 are indicated as formed of No. 30 threads, doubled and spaced 66 ends to the inch.

A fabric formed in this way has the advantage of using fine warp threads closely spaced on the outer surface of the face portion only, saving material and expense by utilizing relatively coarse threads in the other parts of the fabric and by spacing these coarse threads more widely apart. Furthermore, the line of engagement of the fine face portion and the coarse back portion naturally forms a well defined fold line for the fabric.

It will be understood that the fabric is commonly woven in a narrow ware loom, having a compound reed with fine spacing of the reed dents on one side of the dividing line between the fabrics and with relatively coarse spacing of the reed dents on the other side.

In Fig. 4 I have indicated a slightly different construction but one by which substantially similar results may be obtained. The fine face portion 20 and the inside or band portion 21 of the fabric are of the same size and spacing of warp threads as in Fig. 2, previously described, but an intermediate dividing or folding portion 22 is provided between the portions 20 and 21. For the outer part of this intermediate portion 22 I have continued the No. 80 threads as used for the fine face portion of the collar, but these threads are spaced with only 66 ends to the inch, corresponding to the spacing of the coarse warp threads in the band portion 21 of the fabric. The back of the dividing portion is somewhat more loosely woven than either the face or the band portions and contains No. 30 threads, doubled and spaced 33 ends per inch. This dividing portion forms a natural fold for the fabric, owing to its more open spacing.

In Fig. 5, the construction of the face por-

tion 30 and the band portion 31 is similar to that shown in Fig. 2, but the outer part of the intermediate dividing or folding portion 32 is formed of No. 120 warp threads, 5 doubled and spaced 100 ends to the inch, and the rear surface of the part 32 is formed of No. 50 warp threads, doubled and spaced 50 ends per inch. The result of using these extra fine warp threads for the intermediate 10 portion 32 is to provide a natural fold line of appreciable width between the face and the band portions of the fabric.

Having thus described my invention, the advantages thereof will be readily apparent 15 and it will be seen that only one thickness of the face portion of the fabric need be made from the fine and closely spaced warp threads, while the other three portions of the fabric may be of relatively coarse material 20 widely spaced. Furthermore, each of the three fabrics provides a natural fold line and maintains substantially its full strength at the fold line, a marked advantage over certain fabrics heretofore used for 25 this purpose.

Having thus described my invention and the advantages thereof I do not wish to be limited to the details herein disclosed otherwise than as set forth in the claims but what 30 I claim is:—

1. A multiple ply interwoven collar fabric comprising fabric portions of uniform weave throughout and differing from each other in the size of the warp threads therein, said 35 fabric portions at their point of engagement forming a natural fold line for said fabric.

2. A multiple ply interwoven collar fabric comprising fabric portions of uniform weave throughout and differing from each 40 other in size and spacing of the warp threads therein, said fabric portions forming at their point of engagement a natural fold line for said fabric.

3. A multiple ply interwoven collar fabric 45 comprising a face portion having an outer surface with closely spaced fine warp threads and an inner surface with warp threads more widely spaced, and a band portion

formed with relatively coarse warp threads relatively widely spaced.

4. A multiple ply interwoven collar fabric comprising a face portion having an outer surface with closely spaced fine warp threads and an inner surface with coarse warp threads more widely spaced, and a 55 band portion with both inner and outer surfaces having relatively coarse warp threads relatively widely spaced.

5. A multiple ply interwoven collar fabric comprising two distinct longitudinally disposed parallel portions, the outer surface of one portion being formed of closely spaced fine warp threads and the back surface of said portion and all the other portion being formed of coarser warp threads 60 more widely spaced.

6. A multiple ply interwoven collar fabric comprising two distinct longitudinally disposed parallel portions, the outer surface of one portion being formed of closely 70 spaced fine warp threads and the back surface of said portion and all the other portion being formed of coarser warp threads more widely spaced, said fabric having a narrow portion dividing said two parallel 75 portions, and said narrow portion having a face with fine warp threads widely spaced and a back with coarse warp threads also widely spaced.

7. A multiple ply interwoven collar fabric comprising two distinct longitudinally disposed parallel portions, the outer surface of one portion being formed of closely spaced fine warp threads, and the back surface of said portion and all the other portion being formed of coarser warp threads more widely spaced, said fabric 80 having a narrow portion dividing said two parallel portions, and said narrow portion having a face with extra fine warp threads 85 closely spaced and a back with warp threads somewhat finer than the others in the back and widely spaced.

In testimony whereof I have hereunto affixed my signature.

JOHN V. MOORE.